

## UNITED STATES PATENT OFFICE

2,327,977

## QUENCHING OF METALS

Clifford G. van Horst, Hampton Township, Allegheny County, Blaine B. Wescott, Churchill, and Lealle W. Vollmer, Pittsburgh, Pa., assignors to Gulf Research & Development Company, Pittsburgh, Pa., a corporation of Delaware

No Drawing. Application January 12, 1942,  
Serial No. 426,537

6 Claims. (Cl. 148—18)

This invention relates to the quenching of metals; and it is particularly concerned with improved quenching oil compositions comprising a mineral quenching oil and an oil-soluble terpene polymer resin in a controlled amount adequate to substantially increase the initial five second quenching speed without substantially modifying the stress-reducing characteristics of the oil; and it further comprises an improved process of quenching metals comprising preheating the metal to a temperature above its critical temperature and cooling the metal by immersion in a quenching oil bath comprising a light mineral quenching oil and 1.0 to 20.0 per cent of an oil soluble terpene polymer resin; all as more fully hereinafter set forth and as claimed.

While our invention is useful in the quenching of any metal which is advantageously quenched in an oil bath having a high initial quenching speed, it is particularly useful in the quenching of iron base alloys and it will be described hereinafter in detail in connection with the quenching of steel.

Many metal alloys, particularly iron base alloys, such as carbon steels and alloy steels, require heat treatment for the development of maximum properties of hardness and strength. These properties are dependent upon the establishment of certain physical structures in the metallic components of the alloy. In steel, hardenability is determined by the extent to which a martensitic structure is established in the alloy. The production of this structure in steel is usually accomplished by arresting at the desired point, the changes in the internal structure of the alloy which take place during the cooling of the steel from high temperatures. The fact that these physical changes require time for their completion makes it possible to arrest them at the desired point by suitable quick cooling.

Quenching of the steel in aqueous or oil quenching baths is generally used to arrest these physical changes. It is advantageously carried out in such manner that the physical changes in the steel are arrested at or near the point at which maximum hardness is obtained, and is then followed by a tempering treatment involving heating at relatively low temperatures to impart the desired ductility or toughness to the metal at some sacrifice in hardness.

Quenching in aqueous quenching media develops the properties of strength and hardness to the maximum obtainable for a given section of metal. However, quenching in aqueous

quenching media is undesirable in many cases because these media tend to set up excessive amounts of internal stress in the steel resulting in distortion and warping and, in the extreme case, cracking of the quenched piece. As a result, aqueous quenching media have been supplanted by mineral oil quenching media where such mineral oil quenching media have sufficiently high quenching speeds to produce the desired properties in the quenched metal because such mineral oil quenching media are particularly adapted to minimize internal stresses and distortion in the quenched product. This results from the fact that the quenching speeds of mineral oil quenching media are substantially slower than those of aqueous quenching media, due to considerable extent to the formation of a more or less persistent vapor envelope about the quenched piece at the beginning of the quenching cycle, and the fact that in the later stages of the quenching cycle the quenching speeds of mineral oil quenching media are sufficiently slow so that the internal stresses developed in the metal in the early stages of the cycle tend to be relieved. However, since the overall cooling efficiency of the mineral oil quenching media heretofore known is not as great as that of aqueous quenching media, it has been difficult or impossible to effect in mineral oil quenching baths quenching of pieces formed of steels having high critical cooling rates, sufficiently rapidly to develop the properties of strength and hardness to their maximum values or the quenching of pieces having high mass to surface ratios sufficiently rapidly to develop the properties of hardness and strength to the maximum depth. It is desirable therefore to improve the quenching of metals in mineral oil quenching media so that the cooling efficiency in the early stages of the quenching cycle is increased to more nearly approach the cooling efficiency of aqueous quenching media without increasing the quenching speed in the later stages of the cycle sufficiently to deleteriously affect the normal stress-relieving properties of the mineral oil. It is an object achieved by the present invention to provide a method of quenching metals, particularly iron base alloys, in mineral oil quenching media having initial quenching speeds greater than the mineral oil quenching media heretofore known. It is a further object achieved by the present invention to provide mineral oil quenching compositions having cooling efficiencies more nearly approaching the cooling effi-

iciency of water while retaining the stress-preventing characteristics of oil quenches.

The critical cooling rate of a metal is defined as the lowest cooling rate at which maximum hardness is developed. For steel the critical cooling rate is the lowest cooling rate which will produce a full martensitic structure in the steel. Thus it is generally most desirable to effect initial quenching at a speed sufficient to produce a cooling rate at least equal to the critical cooling rate for as great a depth in the metal as possible and to effect the quenching with a minimum of distortion.

The cooling efficiency of a quenching medium is customarily defined in terms of quenching speed and the initial five second quenching speed is a convenient measure of this property of quenching oil compositions, which is the property with which this invention is most concerned. The initial five second quenching speed of a quenching oil composition as referred to throughout this specification and in the appended claims is determined according to the following formula:

Temperature rise in 5 sec. test  
Temperature rise in cold quench test  $\times 100$  - Percent available heat removed in first five sec  
in which the respective values are measured as follows:

Cylindrical test pieces one inch in diameter and 2.5 inches long of stainless steel containing about 18.0 per cent of chromium and 8.0 per cent nickel are heated for one hour at 1500° F. in a furnace equipped with an automatic temperature control. Two quarts of the quenching oil composition to be tested are placed in a calorimeter which has a wire screen positioned in the center of the oil bath to insure constant depth of immersion of the samples. The quenching composition is heated to an initial temperature of 100° F.

One of the preheated test pieces is immersed in the quenching bath by means of light tongs for a period of five seconds without agitation. The test piece is then removed and the bath agitated and the maximum temperature reached is measured. A second preheated test piece is immersed in the bath at an initial temperature of 100° F. and the bath is agitated until the maximum rise in temperature has been produced. The maximum temperature rise measured in this cold quench represents the available heat of the test piece. By substituting the values thus determined for the five second quench and for the cold quench in the above formula a measure of the heat removed in the first five seconds as compared with the total available heat is obtained and is referred to herein as the initial five second quenching speed.

We have discovered that oil-soluble terpene polymer resins have the property, when incorporated in a light mineral oil such as has been used heretofore in the quenching of metals, of substantially increasing the initial five second quenching speed of such an oil without lessening its stress-reducing characteristics, and that by incorporating such terpene polymer resins in mineral quenching oils even in amounts as small as 1.0 per cent substantial increases in the initial five second quenching speeds of the oils can be produced. Furthermore, we have found that the addition of these terpene polymer resins to the mineral quenching oils does not deleteriously affect the stress-relieving properties which normally characterize such oils. By quenching pieces formed of metals having high critical cooling

rates or pieces difficult to quench because of a high ratio of mass to surface, by immersion in quenching oil compositions containing these terpene polymer resins cooling of the metal can be effected at a rate more nearly approaching or equal to the critical cooling rate of the metal without creating excessive stresses in the metal. In this way the hardness of metals having high critical cooling rates can be developed to a degree heretofore unattainable with mineral oil quenching media, and hardening can be effected to a greater depth in pieces having high ratios of mass to surface. Both of these results can be achieved with a minimum of distortion.

The various terpene polymer resins do not increase the initial five second quenching speed of a mineral oil in the same degree. Some are more effective than others and also some are more oil-soluble than others and may be used in larger amounts. We have found also that in most cases the effect of each terpene polymer resin increases directly with the amount used, up to a maximum and then decreases. Consequently, the optimum range of concentration for different terpene polymer resins will differ. In general we have found that amounts of terpene polymer resins between about 1.0 and 20.0 per cent by weight effect substantial increases in the initial five second quenching speed of an oil. By use of the proper resin in suitable amount substantially any initial five second quenching speed between about 20.0 per cent and 37.0 per cent can be obtained. It is possible therefore by suitably compounding quenching oil compositions according to our invention to provide a quenching medium which has an initial five second quenching speed particularly adapted to give best results with the particular metal and the particular type of piece being quenched. For most purposes it is advantageous to use a quenching composition having an initial five second quenching speed of at least about 30.0 per cent and for this reason we find it most advantageous to use the terpene polymer resins in amounts corresponding to at least about 3.0 per cent by weight of the oil.

In compounding the quenching oil compositions of our invention we select for the quenching bath a mineral oil of the type customarily used for quenching steel and other metals and these oils are referred to herein as mineral quenching oils. The oils used for this purpose may be either naphthenic or paraffinic oils and are usually acid treated neutral oils having a viscosity of about 70 to 200 S. U. V. at 100° F., relatively high flash and fire points, and substantial heat stability and resistance to sludging. For optimum results we have found that paraffinic oils which usually have an initial five second quenching speed between about 17.0 and about 19.0 per cent are most advantageous.

We have found also that mixtures of the quenching accelerating agents of our invention may be used. However, in such case, the effect of the respective agents is not entirely additive and the optimum amounts of the respective agents, when used alone, may produce less satisfactory results in mixtures than do somewhat smaller amounts of each agent.

The actual quenching operation using the quenching compositions of our invention is usually carried out by immersion of the preheated metal in the quenching oil composition until sufficient heat has been removed to reduce its temperature

the desired amount. The quenching oil may be used repeatedly with only slight deterioration.

The terpene polymer resins which have been found suitable for the purposes of our invention are such as may be obtained by the polymerization of terpenes such as alpha pinene in the presence of a catalyst such as aluminum chloride, zinc chloride and the like. In commercial production, these polymers are customarily produced by the polymerization of pine extracts such as pine oil, turpentine and related materials. One type of resin which has been found suitable may be prepared by the method described in United States Patent No. 1,938,320 of Samuel W. Cooper, in which a relatively pure high boiling fraction of spirits of turpentine dissolved in an inert solvent is treated at a relatively low temperature with aluminum chloride to effect polymerization, the product is washed with water or dilute hydrochloric acid to remove the catalyst and undesired reaction products, is fractionally distilled and the desired resin fraction is recovered. However, terpene polymer resins obtained by other methods may also be used.

Typical terpene polymer resins which we have found suitable exhibit the following physical properties:

Table I

|                      | Terpene resin B | Terpene resin C |
|----------------------|-----------------|-----------------|
| Melting range (° C.) | 140-150         | 120-130         |
| Ash (per cent max.)  | 0.05            | 0.05            |
| Acid No. (max.)      | 1.0             | 1.0             |
| Saponification No.   | (1)             | (1)             |
| Bromine No.          | 95-100          | 60              |
| Specific gravity     | 0.98            | 0.98            |

<sup>1</sup>Not saponifiable.

The terpene polymer resins when incorporated in amounts of 1.0 to 20.0 per cent in mineral oils such as have been used heretofore in quenching metals produce quenching media having initial five second quenching speeds of at least about 20.0 per cent.

In the following examples there are illustrated specifically several of the more advantageous forms of our invention and the results obtainable thereby.

A terpene polymer resin was prepared according to the method of Cooper U. S. 1,938,320 as follows:

Crude turpentine was distilled through a packed column having an efficiency of approximately 45 plates and a fraction having a boiling range of 155° to 157° C. was recovered. The fraction was mixed with an equal volume of carbon tetrachloride and the mixture was cooled to a temperature less than 1° C. Aluminum chloride in an amount corresponding to about 20 per cent by weight of the turpentine was then added in small increments over a period of 10 minutes so that the temperature, which tended to rise, was maintained relatively close to the starting temperature. The mass was then agitated for a half hour to complete the reaction.

Ice was then added to the reaction mass to destroy any residual aluminum chloride and it was washed several times with caustic soda solution and with water. The washed product was then distilled under 4 cm. vacuum up to 140° C. The terpene resin product remaining after the distillation was used in compounding quenching oils.

Quenching oil compositions were made up by incorporating the resin thus obtained in various

proportions in a neutral paraffinic mineral oil having a viscosity of 100 S. U. S. at 100° F. The initial five second quenching speeds of the respective compositions were then determined as above described and the following results were obtained:

|                                     | Initial five second quenching speed |
|-------------------------------------|-------------------------------------|
| Quenching oil No. 2                 | 16.98                               |
| Quenching oil+2% terpene resin A    | 20.52                               |
| Quenching oil+3.0% terpene resin A  | 21.78                               |
| Quenching oil+5.0% terpene resin A  | 23.57                               |
| Quenching oil+7.5% terpene resin A  | 28.91                               |
| Quenching oil+10.0% terpene resin A | 33.33                               |
| Quenching oil+12.5% terpene resin A | 33.59                               |
| Quenching oil+15.0% terpene resin A | 34.24                               |
| Quenching oil+20.0% terpene resin A | 33.07                               |

In a second series of tests two more highly refined terpene polymer resins having the properties shown above in Table I were used. One was incorporated in varying quantities between 1.0 and 15.0 per cent in a mineral oil such as has been used heretofore in quenching metals and the other was incorporated in corresponding amounts in four different mineral oils suitable for quenching metals. The several mineral oils used in this test had the following characteristics:

|           | Viscosity S. U. S. at 100° F. | Type              |
|-----------|-------------------------------|-------------------|
| Oil No. 1 | 70                            | Neut. paraffinic. |
| Oil No. 2 | 100                           | Do.               |
| Oil No. 3 | 200                           | Do.               |
| Oil No. 4 | 100                           | Naphthenic.       |

The quenching oil compositions made up in this manner were tested for quenching speed and the following results were obtained:

| Resin<br>Per cent by wt. | Initial five second quenching speed |       |       |       |                 |
|--------------------------|-------------------------------------|-------|-------|-------|-----------------|
|                          | Terpene resin B                     |       |       |       | Terpene resin C |
|                          | Oil 1                               | Oil 2 | Oil 3 | Oil 4 | Oil 2           |
| 0.0                      | 17.45                               | 16.98 | 19.01 | 14.99 | 16.98           |
| 1.0                      | 20.31                               | 22.92 | 22.74 |       | 22.27           |
| 2.0                      | 26.25                               | 29.16 | 28.04 | 20.07 | 29.46           |
| 3.0                      | 33.98                               | 33.46 | 31.01 | 26.72 | 34.24           |
| 4.0                      | 35.01                               | 34.11 | 32.16 | 27.56 | 35.28           |
| 5.0                      | 35.79                               | 34.63 | 33.68 | 29.87 | 34.25           |
| 7.5                      | 36.84                               | 35.29 | 33.59 | 29.74 | 35.27           |
| 10.0                     | 36.55                               | 35.42 | 33.33 | 26.87 | 34.11           |
| 12.5                     | 35.52                               | 34.90 | 33.20 | 25.16 | 36.05           |
| 15.0                     | 34.65                               | 34.11 | 30.50 | 22.39 | 34.11           |

As will be seen from these results, by the use of different amounts of different terpene polymer resins, quenching speeds from about 20.0 to about 37.0 per cent are obtainable. Also, it will be noted that in each case the concentration required for the highest quenching speed passes through an optimum range. Also, these resins are substantially less effective with naphthenic oils than with paraffinic oils when used in corresponding amounts.

Hardness and distortion tests were made on pieces of metal quenched in the quenching composition consisting of mineral oil No. 2 and 4.0 per cent of terpene resin B. These measurements were made on specially designed pieces adapted to show, measurably, very small changes in shape due to distortion and having a continuously changing section which permitted measurement of the variation in surface hardenability with varying section of the pieces, and thereby gave an indication of the variation in depth of hardening of the piece. The changes in shape

were measured in inches and the maximum and minimum Brinell hardness occurring at different points on the surface of the piece were determined. Comparative tests were made on pieces quenched in water or in the mineral oil alone.

Results of the distortion measurements are shown in the following table:

| Quenching medium                      | Dimension A | Change in dimension B | Dimension C |
|---------------------------------------|-------------|-----------------------|-------------|
| Tap water.....                        | +0.0134     | +0.0102               | +0.0116     |
| Oil No. 2.....                        | +0.0032     | +0.0024               | +0.0028     |
| Oil No. 2 and 4% terpene resin B..... | +0.0021     | +0.0032               | +0.0028     |

Results of the hardness measurements are shown in the following table:

| Quenching medium                      | Surface Brinell hardness |         |           |
|---------------------------------------|--------------------------|---------|-----------|
|                                       | Minimum                  | Maximum | Variation |
| Tap water.....                        | 649                      | 723     | 74        |
| Oil No. 2.....                        | 361                      | 696     | 335       |
| Oil No. 2 and 4% terpene resin B..... | 645                      | 715     | 70        |

From these results it will be observed that while tap water gives the greatest surface hardness and a variation of only 74 points from the hardest to the softest area, it also gives maximum distortion. The mineral oil alone minimizes distortion, but gives a lowered surface hardening and a variation of 335 points from the maximum to the minimum area indicating a non-uniform depth of hardening throughout the piece. On the other hand, the specimen quenched according to our invention is a quenching oil composition having an initial five second quenching speed of about 35.28 per cent showed distortion as low as that obtained with the plain mineral oil, a surface hardness as high as that obtained with water and a variation in surface hardness no greater than that obtained with water, indicating a depth of hardening approaching to that obtainable with the water quench.

While we have particularly described our invention with reference to certain specific em-

bodiments thereof, it is to be understood that it is not limited to such specific embodiments except as hereinafter defined in the appended claims.

What we claim is:

5. An improved quenching oil composition comprising a mineral quenching oil and at least about 1.0 per cent by weight of an oil-soluble terpene polymer resin.
10. 2. An improved quenching oil composition comprising a mineral quenching oil and an oil-soluble terpene polymer resin in controlled amount adequate to impart to said quenching oil an initial five second quenching speed of at least about 20.0 per cent without substantially modifying the stress reducing characteristics of the oil.
15. 3. A method of quenching metals comprising heating the metal to a temperature above its critical temperature and thereafter cooling the metal by immersion in a quenching oil bath comprising a mineral quenching oil and an amount of an oil-soluble terpene polymer resin, above about 1.0 per cent adequate to impart to the quenching oil bath an initial five second quenching speed of at least about 20.0 per cent.
20. 4. An improved quenching oil composition comprising a solution of at least 3 per cent by weight of an oil soluble terpene polymer resin in a mineral quenching oil.
25. 5. An improved quenching oil composition comprising a mineral quenching oil and an oil soluble terpene polymer resin in controlled amount, adequate to impart to said quenching oil an initial 5 second quenching speed of about 30 to 37 per cent without substantially modifying the stress reducing characteristics of the oil.
30. 6. A method of quenching metals comprising heating the metal to a temperature above its critical temperature and thereafter cooling the metal by immersion in a quenching oil bath comprising a mineral quenching oil and an amount of an oil soluble terpene polymer resin, above about 3 per cent, adequate to impart to the quenching oil bath an initial 5 second quenching speed between about 30 and 37 per cent.

CLIFFORD G. ZUR HORST.  
BLAINE B. WEScott.  
LESLIE W. VOLLMER.